

## UNITED STATES PATENT OFFICE

1,948,245

CHILLED ROLL AND METHOD OF MAKING  
SAME

William H. Seaman, Hammond, Ind.

No Drawing. Application May 3, 1930, Serial No.  
449,688. Renewed December 11, 1933

4 Claims. (Cl. 80—58)

The present invention relates in general to a novel alloy of iron for use in a chilled cast iron roll employed for rolling iron, steel and other metals.

5 One of the objects of the present invention is to provide an alloy iron of such character that when cast in a chilled mold will give throughout the chill depth a scleroscopic hardness of from 90 to 100.

10 Another object is to provide an iron alloy roll in which the chill is of substantially uniform hardness throughout its depth.

Another object is to provide an iron alloy roll in which the depth of the chill may be varied as 15 desired.

A still further object is to provide an iron alloy chilled roll which may be used in cold rolling.

Still another object is to provide a chilled roll 20 of this character which may be substituted entirely for the case hardened forged steel rolls at present employed in cold rolling.

Still another object is to provide an alloy roll of this character which will wear longer, give 25 more uniform results and be very much cheaper than the case hardened steel rolls heretofore necessary for this class of work.

There are other objects of my invention which together with the foregoing will be described in the detailed specification that is to follow.

30 It has been exceedingly difficult heretofore to make a chilled cast iron alloy roll which would be of sufficient hardness to be employed for any cold rolling work. This necessitated the employment of a forged steel case hardened roll which was 35 exceedingly expensive and in which it was difficult to secure uniform hardness throughout the surface of the roll. Furthermore, a case hardened roll of this character is short lived in that as soon as the roll wears sufficiently to penetrate 40 the case hardening, it has to be discarded. Rolls of this character cost as much as \$1.25 per pound. Consequently, in view of the above objections the work done by these rolls was exceedingly expensive. My improved alloy of iron is suitable to 45 be cast in chilled rolls and will give a scleroscopic hardness of from 90 to 100 throughout its chill depth, which may be controlled by modifying the quantity of the constituents employed.

The general characteristic of this iron alloy 50 roll is a very high carbon content, the effect of which is to increase the hardness. There is considerably more graphitic carbon in the gray iron interior of the roll. The roll is also characterized by a high nickel content, which increases the 55 hardness and in combination with the carbon

renders the chill of uniform texture throughout its depth. A very low chromium content is also present, being less than 10% of the nickel. The chromium, in conjunction with the carbon and nickel, produces an alloy which when cast in a 60 chilled mold provides a roll that is exceedingly hard and tough throughout the depth of the chill, as well as being of uniform texture, tough and resilient. Furthermore, the bond between the chill and the gray iron interior is very close.

Of course, in addition to these main constituents there are the usual alloy elements of manganese, silicon, sulphur and phosphorus in suitable proportions. The proportions of the elements of the alloy in addition to iron, to obtain 70 a chilled roll having a scleroscopic hardness from 90 to 100 with the characteristics set forth suitable for substitution in places now requiring forged steel case hardened rolls, are given below:—

|                    | T. C.               | Mn.              | Si.              | S.               | P.               | Cr.              | Ni.                | 80 |
|--------------------|---------------------|------------------|------------------|------------------|------------------|------------------|--------------------|----|
| Hardness 90 to 100 | 3.25<br>to<br>—3.35 | .15<br>to<br>.20 | .15<br>to<br>.25 | .12<br>to<br>.15 | .18<br>to<br>.50 | .25<br>to<br>.35 | 4.75<br>to<br>5.00 |    |
|                    |                     |                  |                  |                  |                  |                  |                    | 75 |

(\*—Carbon may be as high as 3.85 in special instances where more chill and somewhat greater hardness may be required).

85 This alloy is cast in chilled molds in the same mechanical manner as ordinary chilled rolls. The result is a chilled roll having a scleroscopic hardness throughout its chill which is of considerably greater depth than ordinary, of from 90 to 100, and very strong and tough throughout. This 90 roll will wear longer and give better service than forged steel rolls. This follows not only from the hardness of the material of the chill but from its uniformity and depth. The cost of making the cast roll is much less than the 95 cost of a forged steel case hardened roll and since, as outlined above, much better results are secured than with the forged steel roll, the work product is more satisfactory and very much 100 cheaper.

The life of this cast roll is also very much longer and the roll presents innumerable advantages over the forged steel roll, as will be apparent to those skilled in the art. Rolls of this character may be employed for cold rolling 105 wherever it has been necessary heretofore to employ forged steel case hardened rolls.

My invention may be variously modified without departing from the spirit and scope thereof, as set forth in the appended claims.

110

I claim:—

1. The method of making chilled iron alloy rolls which consists in ensuring a chill by using small quantities of silicon, manganese and chromium and securing hardness of said chill by employing carbon and nickel from about 3.25 to about 3.35 carbon and from about 4.75 to about 5.0 nickel.
- 10 2. The method of making chilled iron alloy rolls which consists in ensuring a chill by using small quantities of silicon, manganese and chromium and securing hardness of a varying degree by using carbon and nickel in varying amounts from about 3.25 to about 3.35 carbon and from about 4.75 to about 5.0 nickel.
- 15 3. The method of making chilled iron alloy rolls which consists in ensuring a chill by using small quantities of silicon, manganese and chro-

mium running from about .15 to about .25 silicon and from about .25 to about .35 chromium and from about .15 to about .20 manganese and securing hardness of said chill by using carbon and nickel as desired from about 3.25 to about 3.35 carbon and from about 4.75 to about 5.0 nickel.

4. A chilled iron alloy roll containing small amounts of silicon, chromium and manganese to ensure a chill, said amounts running from about .15 to about .25 silicon and from about .15 to about .20 manganese and from about .25 to about .35 chromium, said roll also containing substantial quantities of carbon and nickel to secure hardness of said chill, said carbon running from about 3.25 to about 3.35 and said nickel running from about 4.75 to about 5.0.

WILLIAM H. SEAMAN.

20

95

25

100

80

105

35

110

40

115

45

120

50

125

55

130

60

135